

# United States Patent [19]

Fromson

[11] 3,865,700

[45] Feb. 11, 1975

[54] **PROCESS AND APPARATUS FOR  
CONTINUOUSLY ANODIZING ALUMINUM**

[76] Inventor: **Howard A. Fromson**, Rogues Ridge Rd., Weston, Conn. 06880

[22] Filed: **May 18, 1973**

[21] Appl. No.: **361,720**

[52] U.S. Cl..... **204/28, 204/211, 204/269**

[51] Int. Cl..... **C23b 5/58, B01k 3/00**

[58] Field of Search ..... **204/28, 211, 267, 269,  
204/58**

[56] **References Cited**

UNITED STATES PATENTS

2,541,275 2/1951 Odier ..... 204/211  
3,471,375 10/1969 Cooke et al. ..... 204/28

FOREIGN PATENTS OR APPLICATIONS

1,005,191 3/1957 Germany ..... 204/28

Primary Examiner—T. M. Tufariello  
Attorney, Agent, or Firm—Burgess, Dinklage &  
Sprung

[57] **ABSTRACT**

Aluminum is continuously anodized using direct current in an anodizing cell having a cathode connected to the source of direct current which is succeeded by a cathodic contact cell having an anode connected to the same source of direct current. The anodizing direct current is introduced into the aluminum in the contact cell, the aluminum having an anodized oxide coating formed thereon in the anodizing cell before entering the contact cell.

**10 Claims, 2 Drawing Figures**



PATENTED FEB 11 1975

3,865,700

FIG. 1.



FIG. 2.



ANODIZING OR OTHER ELECTROLYTIC  
TREATMENT CELL

## PROCESS AND APPARATUS FOR CONTINUOUSLY ANODIZING ALUMINUM

### BACKGROUND

This invention relates to process and apparatus for continuously anodizing aluminum. The term aluminum is used herein to include aluminum base alloys which, like pure aluminum, can be electrolytically anodized to form oxide coatings. More particularly, this invention relates to a technique for continuously anodizing coils or lengths of aluminum, such as aluminum sheets, strips, wire, rods, shapes and the like (hereinafter collectively referred to as aluminum web), by introducing direct current in a cathodic contact cell into an aluminum web passing therethrough having an oxide coating thereon formed in an anodizing cell which precedes the contact cell. The direct current is picked up in the cathodic cell by the already anodized web and is transferred therealong countercurrent to the direction of movement of the web to the anodizing cell in which the oxide coating is formed.

Aluminum and aluminum base alloys in sheet, strip and wire form have been continuously anodized by a number of techniques for many years. Such anodized products are used for electrical and decorative purposes, in the manufacture of household appliances, automotive trim, building materials, farm equipment, furniture, sporting goods, cans, container closures, lithographic plates, transformers, and in many other market and product areas.

Two basic techniques are used to introduce current into a moving aluminum web. The first involves the use of a contact roll or bar and the second is an electrochemical technique utilizing a cathodic contact cell.

The contact roll or bar technique suffers from many deficiencies. For example, the aluminum web must be dry to avoid electrolysis which, if it occurs, dissolves the contact roller or bar anodically leaving pits in the surface thereof. Another problem is arcing between the two surfaces as they become separated which is brought about by the presence of edge burrs or slivers of aluminum on the web surface itself. Arcing causes pitting of the aluminum as well as pitting and oxidation of the contact member itself.

When using the cathodic contact cell technique, one of the limits on how much current can be introduced into the web is the fact that all of the current has to be introduced into a cross-sectional area of the moving web. This causes a surge of current into the unanodized web which is unprotected by an oxide coating. This tends to cause burning and results in the formation of unsound oxide coatings. Up to now the problem of arcing in the use of a solid contact member and the problem of burning due to a surge of current in the contact cell technique have been accepted as inherent limitations in the continuous anodizing of aluminum for the reason that all of the current for the anodizing operation has to be picked up by the moving web in one pass. The reason advanced for this is the fact that the anodic oxide coating formed in the anodizing operation is an electrical insulator.

The present invention now makes it possible to introduce anodizing current into more than one cross-section of the moving aluminum web and imparts to the moving web the means to avoid burning caused by a surge of current into the moving web as it enters the anodizing cell.

### SUMMARY

In its broadest terms, the present invention provides an improvement in a process for continuously electrolytically anodizing aluminum web using direct current. The direct anodizing current is introduced into the aluminum web in a cathodic contact cell, the web having an anodized oxide coating formed thereon before entering the contact cell by the action of the direct current introduced in the contact cell. In a preferred embodiment, anodizing direct current from two or more sources is introduced into the aluminum web in a cathodic contact cell, the strip having an anodized oxide coating formed thereon before entering the contact cell through the action of the direct current introduced in the contact cell itself.

Stated differently, the process of the invention for continuously electrolytically anodizing aluminum web comprises continuously passing an aluminum web through an anodizing cell having a cathode connected to a source of direct current, continuously passing the aluminum web from the anodizing cell into a cathodic contact cell having an anode connected to the same source of direct current, and introducing anodizing direct current into the aluminum strip in the contact cell, the aluminum web having an anodized oxide coating formed thereon in the anodizing cell before entering the contact cell. Preferably, the contact cell has a second anode connected to a second source of direct current and the aluminum web is continuously passed from the contact cell into a second anodizing or other electrolytic treatment cell having a cathode connected to the second source of direct current.

### DESCRIPTION OF THE DRAWING

The present invention will be more fully understood from the following description taken in conjunction with the accompanying drawing wherein:

FIG. 1 is a schematic flow diagram illustrating the features of the invention in its most basic form; and

FIG. 2 is a schematic flow diagram illustrating a preferred embodiment of apparatus for carrying out the process of the invention in a preferred manner.

### DESCRIPTION

The present invention makes it possible to introduce anodizing current into a moving aluminum web into more than one cross-section thereof and into a moving web that already has at least some protective oxide layer formed thereon. This can be accomplished by using a cathodic contact cell, in which the aluminum web is cathodic, between two anodizing cells in which the aluminum strip is anodic, or by utilizing a multiplicity of electrolytic cells in which the aluminum web is alternatively negative or positive. When utilizing the preferred embodiment of the cathodic contact cell between two anodizing cells, the current introduced into the contact cell will travel in both directions thus effectively doubling the current carrying capacity of the moving aluminum web.

Referring now to the drawing and in particular to FIG. 1, the process and apparatus for continuously for electrolytically anodizing aluminum web 12 includes an anodizing cell indicated generally by reference numeral 10 followed by a contact cell indicated generally by reference numeral 20. Each cell includes a suitable tank member 16 for containing an electrolyte 14. The anod-

izing cell 10 has a cathode 18 therein connected to a source of direct current 24. The contact cell 20 has an anode 22 therein which is connected to the same source of direct current 24. The aluminum web 12 continually passes through the anodizing cell 10 followed by the contact cell 20 with the aid of conventional guide rollers positioned as shown in FIG. 1.

The anodizing direct current is introduced into the web 12 in the contact cell 20. The web 12 has an anodized oxide coating formed thereon in the anodizing cell 10 before entering the contact cell 20 by the action of the direct current introduced into the web 12 in the contact cell 20.

FIG. 2 illustrates a preferred embodiment wherein a second anodizing or other electrolytic treatment cell follows the contact cell 20. The second cell 10' contains a cathode 18' which is connected to a second source of direct current 24'. The contact cell 20 contains a second anode 22' which is connected to the same second source of direct current 24'. Thus, by utilizing the preferred embodiment illustrated in FIG. 2 with a contact cell 20 between two anodizing cells 10 and 10', the direct anodizing current introduced into the contact cell 20 from the two separate sources of direct current 24 and 24', travels in both directions thus effectively doubling the current carrying capacity of the moving aluminum web 12. Stated differently, anodizing current is introduced into the web 12 in contact cell 20 from current source 24 which flows in a direction opposite to the direction of movement of the web 12 into the preceding anodizing cell 10 wherein a portion of the desired anodized porous oxide coating is formed. The anodizing operation is completed in anodizing cell 10' by anodizing current from source 24' picked up by the strip 12 and contact cell 20 which is transmitted therealong to the anodizing cell 10'. The web 12 exits from anodizing cell 10' with the desired thickness of porous oxide coating formed thereon.

Instead of a second anodizing treatment in cell 20', which reinforces and adds to the oxide coating formed in cell 20, a further electrolytic treatment wherein the web 12 is positive can be carried out in cell 20'. For example, an electrophoresis operation can be carried out in the embodiment of FIG. 2 in cell 20 whereby resin or lacquer particles are deposited in or on the pores of the oxide coating formed in cell 20.

With respect to the embodiment shown in FIG. 1, the invention can be carried out by passing aluminum web 12 through at least two successive pairs of anodizing cell 10 followed by a contact cell 20.

As is well known in the art, the aluminum web 12 can be cleaned, de-greased or otherwise pretreated using conventional techniques before it reaches the anodizing section and after leaving the anodizing section it can be sealed, dyed or otherwise post-treated using known techniques. The web 12 is passed through the anodizing operation of the invention using conventional winding and feeding equipment.

The present invention will be more fully understood from the following examples which are not intended to limit or otherwise restrict the invention in any way. In the examples, 4 x 8 inch sheets were employed. In all of the examples both sides of the aluminum sheets were anodized and the electrolyte concentration was 230 grams per liter of aqueous sulfuric acid.

### EXAMPLE 1

Aluminum samples were anodized in the sulfuric acid electrolyte at constant electrolyte concentration and temperatures. DC voltage breakdown values were determined and are summarized in Table 1 below:

TABLE 1

|    | CURRENT<br>(in amps) | Time<br>ANODIC<br>(sec.) | Time<br>CATHODIC<br>(sec.) | VOLTAGE<br>BREAKDOWN<br>(volts DC) |
|----|----------------------|--------------------------|----------------------------|------------------------------------|
| 10 | 25                   | 60                       | —                          | 380                                |
|    | 25                   | 60                       | 60                         | 380                                |
|    | 25                   | 60                       | 30                         | 380                                |
|    | 25                   | 30                       | —                          | 290                                |
|    | 25                   | 30                       | 30                         | 290                                |
|    | 25                   | 30                       | 15                         | 290                                |
|    | 20                   | 20                       | 20                         | 220                                |

The results of this Example indicate that reversing the polarity, or passing current through an oxide coating, has no detrimental or adverse effect on the anodized oxide coating. This is indicated by the DC voltage breakdown values which are identical for samples which were subjected to cathodic time and for samples which were not so subjected to cathodic time.

### EXAMPLE 2

Triple sets of aluminum samples were prepared and all were anodized for the same period of time and at the same current density. Set number 1 was anodized only. Set number 2 was anodized and allowed to sit in the electrolyte while the polarity was reversed (samples Cathodic). Set number 3 was anodized and allowed to sit in the anodizing electrolyte without applying any current. For all three sets the anodizing time, the time the polarity was reversed and the time the anodized samples were allowed to sit in the electrolyte was the same.

All of the samples were sealed in boiling water. The weight of the oxide coating formed were determined by first weighing the sample and then stripping off the oxide coating by soaking in a hot chromic-phosphoric acid solution and thereafter re-weighing the sample. The difference in weight divided by the total area of the sample gives the milligrams per square inch of oxide coating on the original sample. The results are summarized in Table 2.

This example illustrates that there is very little difference in the weight of the oxide coating between samples where the polarity was reversed and samples where the anodized samples were allowed to soak in the anodizing electrolyte. This indicates that the loss in oxide weight is due primarily to solvent action of the electrolyte and is not attributable to the passage of current through the coating when the polarity is reversed and the samples are cathodic. In evaluating the data of Table 2 it should be pointed out that the solvent action of the anodizing electrolyte is increased as the temperature increases which accounts for the greater loss in oxide weight at the tests run at higher temperatures.

### EXAMPLE 3

Aluminum samples were anodized following three steps:

1. The sample was anodized at 40°C. at a current density of 50 a/ft<sup>2</sup> for a specific length of time.

2. With the current density remaining at 50 a/ft<sup>2</sup>, the polarity was reversed making the sample cathodic while varying in temperature and time.

pass through a single cross-section of the web. In addition, by utilizing the preferred embodiment illustrated in FIG. 2, the invention makes it possible to minimize

TABLE 2

| TIME<br>(sec) | CURRENT<br>DENSITY<br>(a/ft <sup>2</sup> ) | ACTUAL<br>CURRENT<br>(amps) | VOLTAGE<br>(volts) | "RE-<br>VERSED"<br>VOLTAGE<br>(volts) | TEMP.<br>(°C) | WEIGHT OF                      |                                | WEIGHT OF<br>SET 3<br>(mg/in <sup>2</sup> ) | % WEIGHT LOSS<br>BETWEEN SET<br>1 and 2 |
|---------------|--------------------------------------------|-----------------------------|--------------------|---------------------------------------|---------------|--------------------------------|--------------------------------|---------------------------------------------|-----------------------------------------|
|               |                                            |                             |                    |                                       |               | SET 1<br>(mg/in <sup>2</sup> ) | SET 2<br>(mg/in <sup>2</sup> ) |                                             |                                         |
| 150           | 40                                         | 15.5                        | 16                 | 2                                     | 30            | 5.57                           | 5.45                           | 5.21                                        | 2                                       |
| 150           | 40                                         | 15.5                        | 13                 | 2                                     | 40            | 5.09                           | 4.62                           | 4.67                                        | 9                                       |
| 150           | 40                                         | 15.5                        | 10                 | 2                                     | 50            | 4.56                           | 2.94                           | 3.09                                        | 33                                      |

3. The aluminum sample was again anodized at 40°C. at a current density of 50 a/ft<sup>2</sup> for a specific length of time.

Control samples were anodized at 40°C. at a current density of 50 a/ft<sup>2</sup> for a period of time equaling the total time in steps 1 and 3. Step 2 was eliminated.

All samples in this example were sealed in hot water and the oxide coating weights were determined as described in Example 2. The data are summarized in Tables 3 and 4 below:

TABLE 3

| TIME<br>STEP 1<br>(sec) | VOLTAGE<br>STEP 1<br>(volts) | TIME<br>STEP 2<br>(sec) | VOLTAGE<br>STEP 2<br>(volts) | TEMP<br>STEP 2<br>(°C) | TIME<br>STEP 3<br>(sec) | VOLTAGE<br>STEP 3<br>(volts) | TIME<br>STEP 1<br>& 2 (sec) | SAMPLE<br>COATING<br>WEIGHT<br>(mg/in <sup>2</sup> ) | CONTROL<br>COATING<br>WEIGHT<br>(mg/in <sup>2</sup> ) | % WEIGHT<br>LOSS OF<br>SAMPLE |
|-------------------------|------------------------------|-------------------------|------------------------------|------------------------|-------------------------|------------------------------|-----------------------------|------------------------------------------------------|-------------------------------------------------------|-------------------------------|
| 54                      | 13.5                         | 48                      | 2                            | 60                     | 66                      | 13                           | 120                         | 4.488                                                | 4.946                                                 | 9.26                          |
| 54                      | 13.0                         | 48                      | 2                            | 50                     | 66                      | 13                           | 120                         | 4.496                                                | 4.804                                                 | 6.41                          |
| 54                      | 13.0                         | 48                      | 2                            | 40                     | 66                      | 13                           | 120                         | 4.867                                                | 5.013                                                 | 2.90                          |
| 54                      | 13.0                         | 48                      | 2                            | 40                     | 66                      | 13                           | 120                         | 4.788                                                | 4.875                                                 | 1.78                          |
| 108                     | 13.5                         | 96                      | 4                            | 60                     | 132                     | 13                           | 240                         | 7.229                                                | 9.229                                                 | 21.67                         |
| 108                     | 13.5                         | 96                      | 2                            | 50                     | 132                     | 13                           | 240                         | 8.179                                                | 9.329                                                 | 12.32                         |
| 108                     | 13.0                         | 96                      | 2                            | 40                     | 132                     | 13                           | 240                         | 8.558                                                | 2.279                                                 | 7.77                          |

TABLE 4

| TOTAL<br>AMPERE-<br>MIN | TEMP<br>STEP 2<br>(°C) | WEIGHT<br>OF SAMPLE<br>(mg/in <sup>2</sup> ) | WEIGHT OF<br>CONTROL<br>(mg/in <sup>2</sup> ) | % WEIGHT LOSS<br>OF SAMPLE vs.<br>CONTROL |      |
|-------------------------|------------------------|----------------------------------------------|-----------------------------------------------|-------------------------------------------|------|
|                         |                        |                                              |                                               | CONTROL                                   |      |
| 100                     | 60                     | 4.488                                        | 4.946                                         | 9.26                                      |      |
| 100                     | 50                     | 4.496                                        | 4.804                                         | 6.41                                      |      |
| 100                     | 40                     | 4.788                                        | 4.875                                         | 1.78                                      | 2.34 |
| 100                     | 40                     | 4.867                                        | 5.013                                         | 2.90                                      |      |
| 200                     | 60                     | 7.229                                        | 9.229                                         | 21.67                                     |      |
| 200                     | 50                     | 8.179                                        | 9.329                                         | 12.32                                     |      |
| 200                     | 40                     | 8.558                                        | 9.279                                         | 7.77                                      |      |
| 320                     | 60                     | 8.304                                        | 13.942                                        | 40.43                                     |      |
| 320                     | 50                     | 10.729                                       | 14.025                                        | 23.50                                     |      |
| 320                     | 40                     | 12.817                                       | 13.984                                        | 8.34                                      |      |

It is known that anodic oxide requires a forming voltage of somewhere between 12 and 13 volts (cf. *Finishing Of Aluminum*, Wernick and Pinner). The foregoing Examples demonstrate that when the polarity is reversed and the anodized aluminum samples are made the negative or cathodic pole of the cell, the anodized samples exhibit an unusual phenomenon and at the same current density used to anodize, the voltage drops to between 1 and 2 volts. Only minor heat is generated by resistance and there is practically no weight loss as demonstrated herein. This unique property makes it possible to continue to introduce or feed current into the aluminum web at portions where the anodic oxide coating has already been formed. By using this technique, it now becomes possible to continuously DC anodize aluminum webs without the limitations imposed by the contact roll method or the standard contact cell method where all of the current is introduced in one

55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
61

plating techniques to thereafter deposit one or more electroplated metal layers on the aluminum web, for example, even using conventional contact drums and the like.

What is claimed is:

1. In a process for continuously electrolytically anodizing aluminum, the improvement which comprises introducing anodizing direct current into said aluminum in a cathodic contact cell having therein an anode connected to said source of direct current, said aluminum having an anodized oxide coating formed thereon before entering said cell through the action of the direct current introduced in the contact cell itself.

2. In a process for continuously electrolytically anodizing aluminum, the improvement which comprises introducing anodizing direct current from two or more sources in a cathodic contact cell having therein anodes connected to said sources of direct current, the aluminum having an anodized oxide coating formed thereon before entering said cell through the action of the direct current introduced in the contact cell itself.

3. Process for continuously electrolytically anodizing aluminum web which comprises continuously passing said web through an anodizing cell having therein a cathode connected to a source of direct current, continuously passing said web from said anodizing cell into a cathodic contact cell having therein an anode connected to said source of direct current, and introducing anodizing direct current into said web in said contact cell, said web having an anodized oxide coating formed thereon in said anodizing cell before entering said contact cell through the action of the direct current introduced in the contact cell itself.

4. Process of claim 3 wherein said contact cell has a

second anode connected to a second source of direct current and said web is continuously passed from said contact cell into a second cell having a cathode therein connected to said second source of direct current.

5. Process of claim 4 wherein said second cell is an anodizing cell.

6. Process of claim 4 wherein said second cell is a further electrolytic treatment cell.

7. Process of claim 3 wherein said aluminum strip is passed through at least two successive pairs of said anodizing cell followed by said contact cell.

8. Apparatus for continuously electrolytically anodizing aluminum web which comprises anodizing cell means containing a cathode connected to a source of direct current, cathodic contact cell means containing an anode connected to said source of direct current, and means for continuously passing said aluminum web first through said anodizing cell means and then through said contact cell means, the anodizing direct current entering said web in said contact cell means with an anodized oxide coating formed thereon through the action of the direct current introduced in the contact cell itself.

9. Apparatus of claim 8 wherein said contact cell means contains a second anode connected to a second source of direct current and a second cell means are provided containing a cathode connected to said second source of direct current, said means for passing being adapted to continuously pass said web through said second anodizing cell means after passing through said contact cell means.

10. Apparatus of claim 9 wherein said second cell means is an anodizing cell means.

\* \* \* \* \*

UNITED STATES PATENT OFFICE  
CERTIFICATE OF CORRECTION

Patent No. 3,865,700 Dated February 11, 1975

Inventor(s) Howard A. Fromson

It is certified that error appears in the above-identified patent and that said Letters Patent are hereby corrected as shown below:

Column 1, line 39 "arching" should read --arcing--;

Column 3, line 8 "curret" should read --current--;

Column 4, line 36 "andizing" should read --anodizing--.

Column 5, line 50 after Table 4 insert:

--Note: Ampere - min. = time anodized x current density.

C.D. = 50 a/ft<sup>2</sup>

Anodizing Temperature = 40°C.--

Signed and sealed this 24th day of June 1975.

(SEAL)

Attest:

RUTH C. MASON  
Attesting Officer

C. MARSHALL DANN  
Commissioner of Patents  
and Trademarks